

1,185,220.

W. H. LUHRS,  
METHOD OF FORMING REINFORCED BEARINGS,  
APPLICATION FILED APR. 23, 1915.

Patented May 30, 1916.



Witnesses

W. H. Ford  
James P. Barry

William H. Luhrs Inventor

By Whittier, Hubbell & Whittier

Attorneys

# UNITED STATES PATENT OFFICE.

WILLIAM H. LUHRS, OF DETROIT, MICHIGAN

## METHOD OF FORMING REINFORCED BEARINGS.

1,185,220.

Specification of Letters Patent. Patented May 30, 1916.

Application filed April 23, 1915. Serial No. 23,315.

To all whom it may concern:

Be it known that I, WILLIAM H. LUHRS, a citizen of the United States of America, residing at Detroit, in the county of Wayne 5 and State of Michigan, have invented certain new and useful Improvements in Methods of Forming Reinforced Bearings, of which the following is a specification, reference being had therein to the accompanying drawings.

The invention relates to the manufacture of bearings which are provided with babbitted or soft metal wearing surfaces, and it is the object of the invention to reduce the 15 cost of manufacture and at the same time to obtain a product which is more durable than those heretofore used.

In the construction of babbitted bearings it is usual to produce sufficient depth of the 20 Babbitt metal to compensate for wear, but in addition to this it is also usual to provide a much greater depth to increase the strength of the bearing. This is for the reason that the friction upon the bearing surface will tend to displace the metal in relation to the outer case and unless there is sufficient body to resist these stresses the Babbitt lining may become detached, thereby 25 destroying the bearing. With certain constructions the babbitt is mechanically united to its holder by perforating the latter so as to form interlocking studs, but the union is an imperfect one and sooner or later the soft metal becomes loosened and is eventually 30 destroyed. Thus to guard against such a result the depth of the soft metal is made greater than would be required for merely compensating for wear. With the present invention I have obtained a greatly improved bearing, first, by reinforcing the soft metal with a rigid metal, such as steel, and second, by integrating the contacting surfaces of the soft and harder metal so that 35 they become in effect a unit, and the depth of the soft metal may therefore be restricted to that necessary for wear.

In carrying out my improved process for manufacturing bearings it is essential, first, to prepare the surface of the reinforcing metal so that it will be integrated with the soft or Babbitt metal. This I preferably accomplish by subjecting the reinforcing metal to a series of treatments preliminary to a

tinning process by which the surface is coated with metallic tin. After the tinning process the reinforcement is heated to a pre-determined temperature, and the Babbitt metal is then cast thereupon, with a result that it will be completely molecularly united with the reinforcement and will become a unit therewith.

In the drawings, I have illustrated a few of the specific forms of bearing resulting from my process, in which—

Figure 1 is a perspective view showing one construction, and Fig. 2 a longitudinal section through a modified construction and Fig. 3 shows in longitudinal section the most simple form of the invention.

A is the metallic reinforcement, preferably formed of sheet steel, pressed or otherwise fashioned into the desired form. This reinforcement is first treated by dipping the same in a solution of substantially the following composition: 100 pounds of muriatic acid, 1 ounce of salammoriae, cut with 2 ounces of aluminum. The reinforcement being first heated to a temperature of 200° F., is then plunged into this solution and is allowed to cool. The next treatment is the immersing of the pre-heated metal in a solution composed of substantially: 100 pounds of muriatic acid, cut with 5 ounces of zinc. After immersing in this solution the bearing is again allowed to cool. The next treatment is the immersing of the pre-heated metal in a solution composed of: 100 pounds of muriatic acid and 8 ounces of zinc, and after withdrawing from the solution the metal is plunged into a molten tin bath, with a result that the surface will be completely coated with tin. The reinforcement is then permitted to cool, after which it is re-heated to substantially 450° F., and is then assembled in proper position for casting the Babbitt metal thereon.

As shown in Fig. 1, the Babbitt metal is cast so as to have a portion B extending parallel to the reinforcement A, and portions C and C' extending around the end of said reinforcement. Thus the wearing surface for both radial and end thrust is formed of the softer metal.

In Fig. 2 a modified construction is shown, in which flanges D are united to the tin surface of the ends of the reinforcement A, and

the babbitt E is cast to extend parallel to both the reinforcement and the flanged portions.

My novel process may be utilized in the manufacture of various specific structures.

What I claim as my invention is:—

1. The process of forming reinforced Babbitt or soft metal bearings, comprising the treatment of the reinforcing metal to a series of acid baths having small proportions of metallic salts therein, the plunging of the metal after treatment into a molten tin bath, and the casting of the babbitt upon the tin surface to become molecularly united thereto.

2. The process of forming reinforced Babbitt or soft metal bearings, comprising the treatment of the reinforcing metal by first immersing in a bath of muriatic acid and aluminum salt, second, in immersing in a bath of muriatic acid and zinc salt, third,

in immersing in a bath of muriatic acid with a greater proportion of zinc salt, fourth, in immersing in molten tin, and fifth, in casting the Babbitt metal upon the tin surface to become molecularly united thereto.

3. The process of forming reinforced Babbitt or soft metal bearings, comprising the treatment of the reinforcing metal to a series of acid baths containing metallic salts, the plunging of the metal after treatment into a bath of molten metal, such as will molecularly unite with the babbitt, and the casting of the babbitt upon the coated surface.

In testimony whereof I affix my signature in presence of two witnesses.

WILLIAM H. LUHRS.

Witnesses:

JAMES P. BARRY.

ARTHUR D. PULVER.